

## UNITED STATES PATENT OFFICE

2,030,357

PROCESS OF REMOVING TIN FROM  
COLUMBIUM ALLOYSErnest F. Doom, Niagara Falls, N. Y., assignor,  
by mesne assignments, to Union Carbide and  
Carbon Corporation, a corporation of New YorkNo Drawing. Application March 21, 1934.  
Serial No. 716,651

3 Claims. (Cl. 75—18)

The present invention relates to a process of treating metallic alloys and more particularly to a process of treating alloys of columbium for the removal and separation of tin.

5 Naturally occurring columbium ores such as columbite are frequently associated with stanniferous minerals. If such tin-contaminated ores are smelted for the production of alloys of columbium with iron, silicon, or other metals, a major portion of the tin content of the ore will ordinarily be recovered in the columbium alloy. For certain uses to which the columbium alloys are put, notably as a means of introducing columbium into steel, a high tin content is often desirable. 10 The removal of the associated tin from columbite prior to smelting is rarely feasible in a commercial manner, when known methods of ore dressing are resorted to, and where a fairly complete removal of tin is desired. Special chemical treatments of the ore have been used heretofore, but 15 all of them are relatively expensive.

It is an object of my invention to provide a means of cheaply and relatively completely removing tin from columbium alloys.

20 I have found that if silicon is incorporated in a tin-containing columbium alloy in an amount exceeding a silicon to columbium ratio of about 1 to 6.5, the tin content thereof may be leached out by means of hydrochloric acid or a similar acid. It appears probable, from my investigations, that when the silicon content of the alloy is less than this ratio the tin is combined with the columbium as an acid-insoluble compound. When the silicon content of the alloy exceeds this 25 ratio, the tin is in a free or at least in a soluble form. This silicon-columbium ratio roughly corresponds with the silicide  $\text{Cb}_2\text{Si}$ , and it may well be that the relative affinity of columbium for silicon is greater than the affinity of columbium for tin, so that, when sufficient silicon is present to form the silicide, the tin is left in a free or soluble form. It will be understood, however, that this is merely a theoretical explanation and that this invention does not depend upon the correctness of this theory. The presence of other silicide-forming elements in the alloy may alter the minimum ratio of silicon to columbium necessary for the best extraction of tin. In general I 30 prefer to use somewhat more silicon in the alloy

than the ratio shown, this being considered more conducive to an easy solution of the tin.

In carrying out my process, columbium alloys which may be produced by smelting stanniferous columbium oxide ores, by using any suitable reducing agent such as carbon, aluminum, or silicon, may be treated for the elimination of tin. The required silicon content of the alloy may be obtained by the reduction of silica, simultaneously with the reduction of the columbite ores, either 10 of silica naturally occurring in the ore, or of silica which may be intentionally added to the ore. Alternatively, a silicon-columbium alloy may be obtained by directly alloying a columbium alloy with metallic silicon. 15

The alloy produced by any of the above described processes is then comminuted and treated with a leaching agent. A leaching agent which has been found to be particularly suitable for the purposes of this invention is hydrochloric acid. However, other acidic agents, and particularly acids having substantially the same degree of dissolving action, may be used. The treatment will usually require several hours, depending on the amount of tin to be extracted, the temperature, the concentration of the acid, and the size of the alloy particles being treated. I have found that the tin can be practically completely extracted when the alloy is comminuted so that the particles will pass a 20 mesh screen, (1/16" opening), the particles being treated with hydrochloric acid of about 11° Baumé. The acid treatment will frequently dissolve small amounts of some of the alloy constituents other than tin, such as iron, but I have found that very little, 35 if any, loss of columbium occurs. The concentration of acid is not critical, as I have employed dilute and concentrated acid with practically equal success. In general, an excess of acid of fair concentration is to be preferred, as it has- 40 tens solution of the tin.

In practicing my invention, three lots of ferro-columbium-silicon alloy containing varying ratios of silicon to columbium were comminuted to 20 45 mesh and treated for 36 hours with a solution of about equal volumes of hydrochloric acid (20° Bé.) and water. In each case the proportions were such that one part of alloy was treated with two parts of the diluted acid. The results 50

of this treatment are indicated in the following table:

Alloy No. 1

|              | Before treatment           | After treatment |
|--------------|----------------------------|-----------------|
| Cb.          | 43.29%                     | 45.79%          |
| Ta.          | 19.33                      | 20.47           |
| Si.          | 3.03                       |                 |
| C.           | 0.62                       |                 |
| Sn.          | 8.45                       | 8.62            |
| Balance.     | Largely iron<br>1 to 14.28 |                 |
| Ratio Si:Cb. |                            |                 |

Alloy No. 2

|              | Before treatment          | After treatment |
|--------------|---------------------------|-----------------|
| Cb.          | 46.48%                    |                 |
| Ta.          | 0.77                      |                 |
| Si.          | 7.23                      |                 |
| C.           | 0.04                      |                 |
| Sn.          | 1.24                      | 0.49%           |
| Balance.     | Largely iron<br>1 to 6.42 |                 |
| Ratio Si:Cb. |                           |                 |

Alloy No. 3

|              | Before treatment          | After treatment |
|--------------|---------------------------|-----------------|
| Cb.          | 40.42%                    | 45.03%          |
| Ta.          | 16.08                     | 17.91           |
| Si.          | 16.64                     |                 |
| C.           | 0.62                      |                 |
| Sn.          | 3.26                      | 0.08            |
| Balance.     | Largely iron<br>1 to 4.43 |                 |
| Ratio Si:Cb. |                           |                 |

35 It will be noted that where the silicon-colum-

biun ratio is nearly 1 to 6.5, a substantial amount of the tin is removed by the treatment. With a silicon content below this ratio, as in Alloy No. 1, the tin is completely insoluble, whereas with a higher silicon content, as in Alloy No. 3, the tin is substantially all removed by the acid treatment.

The columbium alloy treated by my process for the elimination of tin may be used directly for adding columbium to other metals, such as steel, or if a lower silicon alloy is desired the silicon may be removed or lowered by any of the conventional refining processes prior to such use.

What I claim is:

1. The process of removing tin from columbium alloys which comprises introducing silicon into said alloys in an amount at least equivalent to that required to provide a ratio of silicon to columbium satisfying the formula  $Cb_2Si$ , and treating said alloys with aqueous hydrochloric acid.

2. The process of reducing the proportion of tin in tin containing columbium alloys, which comprises introducing silicon into such alloy in an amount at least equivalent to a silicon to columbium ratio of about 1 to 6.5, comminuting the silicon-containing alloy and leaching it with a solution of hydrochloric acid.

3. The process of reducing the proportion of tin which is contained in an iron-columbium alloy, which comprises introducing silicon into said alloy in a ratio of about 1 to 6.5, comminuting the alloy, and leaching it with aqueous hydrochloric acid.

ERNEST F. DOOM. 35

CERTIFICATE OF CORRECTION.

Patent No. 2,030,357.

February 11, 1936.

ERNEST F. DOOM.

It is hereby certified that error appears in the printed specification of the above numbered patent requiring correction as follows: Page 1, first column, line 14, for "desirable" read undesirable; and that the said Letters Patent should be read with this correction therein that the same may conform to the record of the case in the Patent Office.

Signed and sealed this 17th day March, A. D. 1936.

Leslie Frazer

Acting Commissioner of Patents.

(Seal)

CERTIFICATE OF CORRECTION.

February 11, 1936.

Patent No. 2,030, 357.

ERNEST F. DOOM.

It is hereby certified that error appears in the printed specification of the above numbered patent requiring correction as follows: Page 1, first column, line 14, for "desirable" read undesirable; and that the said Letters Patent should be read with this correction therein that the same may conform to the record of the case in the Patent Office.

Signed and sealed this 17th day March, A. D. 1936.

Leslie Frazer

Acting Commissioner of Patents.

(Seal)